

1

2,907,714

## WATER-IN-OIL LUBRICANT AND HYDRAULIC FLUID

Charles E. Francis and John J. Weaver, Martinez, Calif., assignors to Shell Development Company, New York, N.Y., a corporation of Delaware

No Drawing. Application July 12, 1957  
Serial No. 671,405

9 Claims. (Cl. 252—33.3)

This invention relates to improved emulsion lubricants and hydraulic fluids. More particularly, it pertains to water-in-oil emulsion lubricants especially useful for slow speed diesel engines and as fire-resistant hydraulic fluids which possess good lubricating properties and which are stable, non-corrosive and wear-resistant.

Although it is known in the art that certain emulsions are useful as coolants and lubricants in metal working operations and as rust and corrosion inhibitors, their use as engine lubricants and as hydraulic fluids has been limited. Under engine operating conditions, emulsions generally lack desired lubricity and cause wear and corrosion.

Fluid compositions for use in many hydraulic systems should be fire-resistant and non-corrosive. They should be capable of preventing wear and be thermally stable and resistant to oxidation. Various compositions have been proposed for use as hydraulic fluids, but none of them are entirely satisfactory. Thus, mineral oils are highly flammable, castor oil results in sludge and gum formation, esters of carboxylic acids cause swelling of rubber, the organic phosphates and the glycols are corrosive, the halogen-containing materials tend to hydrolyze to produce corrosive materials, emulsion lack wear resistant properties, while the silicone compounds lack lubricity and present a health hazard.

It is an object of this invention to provide a emulsion lubricant and fire-resistant hydraulic fluid having good lubricating properties. Another object is to provide a fluid which is a satisfactory lubricant for low speed diesel engines and hydraulic equipment, which is stable, fire-resistant, resistant to deterioration, inhibits corrosion and does not cause wear. Still another object of this invention is to provide an emulsion lubricant and fire-resistant hydraulic fluid of good lubricating quality even when subjected to various adverse conditions of temperature, loads and speeds as encountered in various diesel engines operating on high sulfur fuels or in certain hydraulic systems.

These and other objects are accomplished in accordance with this invention by providing a water-in-oil emulsion which is from about 20 to about 45% water phase and from about 55% to about 80% oil phase, the emulsion containing a combination of minor amounts of three essential additives, namely (1) an oil-soluble basic polyvalent metal aromatic carboxylate, (2) an oil-soluble basic polyvalent metal organic sulfonate, the metals of

2

both compounds being of group II metals of the periodic table and having an atomic number of from 12 to 56, and (3) an oil-soluble chlorohydrocarbon thiocarbonate ester.

The oil-soluble basic polyvalent metal aromatic carboxylates of the group II metals of the periodic table having an atomic number of from 12 to 56, inclusive, and preferably the alkaline earth metals, include such compounds as basic calcium, barium, magnesium, strontium and zinc salts of hydrocarbon substituted benzoic, salicylic, resorcylic, anthranilic and naphthoic acids such as the basic calcium, barium, magnesium and/or zinc salts of  $C_3-C_{22}$ -alkylbenzoic,  $C_8-C_{22}$ -alkylsalicylic,  $C_3-C_{22}$ -alkynaphthoic acids and mixtures thereof.

The preferred salts are the basic barium, calcium, magnesium, and zinc salts of laurylsalicylic acid, or of stearyl salicylic acid or of a mixture of alkylsalicylic acids in which the alkyl groups contain from 8 to 30, preferably 14 to 22, carbon atoms. The basic calcium salts of these alkylsalicylic acids are particularly preferred. The highly basic salts may be prepared, for example, by the processes described in U.S. Patents 2,409,687 or 2,616,910.

The sulfonates are oil-soluble basic polyvalent metal organic sulfonates, of which petroleum sulfonates of the metals of group II of the periodic table having an atomic number of from 12 to 56, inclusive, are preferred, and especially of the alkaline earth metals. Suitable sulfonates include the basic calcium, barium, magnesium and zinc petroleum sulfonates of oil-soluble petroleum sulfonic acids. The acids should range in molecular weight from about 350 to 550 and preferably are in the range of from 400 to 500. Other sulfonates include the oil-soluble basic calcium, barium, magnesium and zinc tertiarybutylnaphthalene sulfonates, dinonyl naphthalene sulfonates, diwaxbenzene sulfonates, waxphenol sulfonates and mixtures thereof.

By a basic salt as used with reference to the aromatic carboxylates and the sulfonates is meant that the amount of metal neutralizing agent, e.g. metal oxide, metal hydroxide, or metal carbonate, used is in excess of that stoichiometrically required to neutralize the carboxylic or sulfonic acid to produce the normal salt. The excess basicity of the salts used in compositions of this invention should be from 25% to 1000% and preferably from about 50% to 800%.

The oil-soluble chlorohydrocarbyl hydrocarbylthiocarbonate ester, preferably a polychloroalkyl hydrocarbylthiocarbonate, may be represented by the formula



where the Y's are S or O atoms, at least one being a sulfur atom,  $n$  is a whole number which is no more than twice the number of carbon atoms in  $R'$ , preferably it is no more than the same as the number of carbon atoms in  $R'$  and still more preferred that it be of the order of one-half of the number of carbon atoms in  $R'$  being at least 4, and  $R$  and  $R'$  are hydrocarbon radicals containing a total together of at least 12 carbon atoms, at least one of them and preferably  $R'$  being an aliphatic hydrocarbon radical of at least 10 carbon atoms, preferably from 12 to 30 carbon atoms and having at least four substituent chlorine atoms.

These chlorohydrocarbyl thiocarbonate esters are suitably prepared by the reaction of polychlorohydrocarbons with less than the stoichiometrically equivalent amount of an alkali metal or of an alkaline earth metal hydrocarbyl thiocarbonate, with the formation of the alkali metal or alkaline earth metal halide and the thiocarbonate ester.

The thiocarbonate may be a mono-, di- or tri-thiocarbonate. Accordingly for the preparation of the ester, various alkali metal or alkaline earth metal hydrocarbyl thiocarbonates can be suitably used, such as the sodium, potassium, calcium and barium hydrocarbylxanthates (a thionothiolcarbonate) and corresponding mono- or tri-thiocarbonates. Illustrative suitable substances are alkali metal lower alkyl xanthates, such as sodium methyl xanthate, potassium methyl xanthate, potassium ethyl xanthate, potassium butyl xanthate, sodium amyl xanthate, and potassium amyl xanthate and alkali metal lower aralkyl xanthates, such as potassium benzyl xanthate. The mono- and tri-thiocarbonate ester salt reactants are illustrated by the substances more simply designated by their formulae:



and corresponding other ester-salts containing hydrocarbon radicals of from 1 to 7 carbon atoms.

The thiocarbonate ester-salts are suitably reacted with various polychlorinated hydrocarbons in such proportions as to leave at least four chlorine atoms in the resulting thiocarbonate full ester. The polychlorinated hydrocarbons are preferably polychlorinated aliphatic hydrocarbons of from about 2 to about 30 carbon atoms per molecule. Mixtures of polychloroalkanes, including cyclic and acyclic alkanes, are particularly useful. Some readily available materials which may be used are chlorinated naphtha, chlorinated paraffinic lubricating oils, chlorinated paraffin wax and chlorinated rubber.

As indicated, the reactants are reacted in proportions such that the final product contains both chlorine and thiocarbonate groups. The amounts of chlorine and sulfur in the final product can vary over a wide range such as from about 25 to about 40% by weight chlorine and from about 7 to about 15% by weight sulfur.

An illustrative product of this type can be prepared as described in the following example:

#### EXAMPLE I

Petroleum naphtha (Stoddard solvent) was chlorinated by bubbling chlorine gas through it until it contained about 52% by weight of chlorine. 225 parts by weight of the chloronaphtha was mixed with about 400 parts of acetone and 100 parts of potassium amyl trithiocarbonate. The mixture was refluxed with stirring on a water bath and heated for about one and one-half hours, after which it was cooled and filtered to remove the potassium chloride. The acetone was removed by distillation, after which benzene was added and distilled off to insure removal of water from the product. The resulting product was a bright liquid, soluble in oil, and a typical analysis showed a chlorine content of 35% and a sulfur content of about 10%, or a trithiocarbonate (divalent  $\text{CS}_3$ ) content of about 11.3%.

Similar polychloronaphtha alkyl xanthates are marketed by the Monsanto Chemical Company under the name "Santopoid S." A typical "Santopoid S" (polychloronaphtha alkyl xanthate) has the following characteristics: sp. gr. 1.19 at 60°/60° F.; flash point 250° F.; viscosity 63 cs. at 100° F.; sulfur 11%; chlorine 31%.

These three essential additives are used each in an amount of from about 0.5% to about 12% by weight and preferably the two basic salts are used in amounts from

about 2% to about 4% while the chlorohydrocarbyl thiocarbonate compound is used from about 3% to about 10% by weight, based on the amount of oil in the emulsion.

In addition to the above three essential additives and mixtures thereof it is preferred to use in such compositions small amounts of from about 0.01% to about 2%, preferably from about 0.2% to about 1% of phenolic, amine and/or metal thiophosphate anti-oxidants such as alkyl phenols, e.g., di- and trialkyl phenols, for instance 2,4-, 2,3-, 3,4-, 2,6- and 3,5-diamylphenol, 2,4-dimethyl-6-tert.butylphenol, 2,6-ditert.butyl-4-methylphenol; arylamines such as phenyl-alpha-naphthylamine or phenyl-beta-naphthylamine; metal thiophosphates such as calcium or zinc dimethyl cyclohexyldithiophosphate; dyes such as various oil-soluble dyes e.g. Naphthol yellow, Sandoz yellow, methylene blue, alizarin compounds etc.; anti-foaming agents e.g., silicone polymers (DC-200 fluids ranging in viscosity in centistokes from 100 to 1000 at 250° C.) or silicone type A fluid made by Dow Corning Co. and described in U.S. Patents 2,563,588 and 2,662,055 and mixtures thereof.

The aqueous phase of the water-in-oil emulsion should range from about 20% to about 45% and preferably from about 30% to about 40% by weight of the emulsion. The oil phase containing the additives comprise the balance of the emulsion. The oil may be entirely a hydrocarbon oil of wide viscosity range, e.g., from less than 50 SUS at 100° F. to 150 SUS at 210° F. Oils of this type can be obtained from various crudes such as paraffinic, naphthenic or mixed base crudes; refined oils in the lubricating oil viscosity range are preferred. On the other hand, the hydrocarbon oil may be blended with fixed oils such as castor oil, lard oil and the like and/or with synthetic lubricants such as polymerized olefins, organic esters of organic and inorganic acids, e.g., di-2-ethylhexyl sebacate, diethyl phthalate, triethyl phosphate; polymeric tetrahydrofuran, polyalkyl silicone polymer, e.g., dimethyl silicone polymer and the like. Where mixtures or blends are used the hydrocarbon oil such as a mineral lubricating oil is always present in the predominant amount such as from about 60% to about 95% of the oil blend.

A straight mineral lubricating oil, having a viscosity index of at least 50 and ranging in viscosity at 100° F. of from 75 to 400 SUS, is usually preferred. When it is derived from a lubricating oil stock of low viscosity index it is readily provided as raffinate in a selective solvent extraction process as is well understood in the art. The emulsion can be prepared by adding the required amount of water to an oil containing the three essential additives, namely an oil containing the two base salts and the thiocarbonate-containing compound, while constantly stirring the mixture. Heating the emulsion during or after it is prepared is not necessary. If desired, the emulsion can be homogenized to insure a homogeneous composition. Instead of making the finished emulsion, the oil concentrate containing the essential additives namely the two basic salts and the chlorohydrocarbyl thiocarbonate compound can be prepared and the required amount of water added when the emulsion lubricant is ready for use. In this way storage and shipping costs can be greatly reduced.

A finished emulsion fluid [composition (A)] of the invention was prepared by slowly adding 40% water to a vessel containing 2% each of oil-soluble basic calcium petroleum sulfonate (180% excess base) and oil-soluble basic calcium  $\text{C}_{18-22}$  alkyl salicylate (50% excess base) and 5% additive Example I dispersed in 51% mineral oil of 100 SUS at 100° F. The entire mixture was passed through a colloid mill where it was agitated until a homogeneous water-in-oil emulsion was formed. A similar composition (A') was prepared but instead of using a colloid mill to form a homogeneous emulsion, a homogenizer was used.

Other compositions which illustrate emulsions of this invention are:

|                                                                     | Percent wt.<br>Additive<br>in Total<br>Emulsion | Percent wt.<br>of Additive<br>in Oil |
|---------------------------------------------------------------------|-------------------------------------------------|--------------------------------------|
| Composition B:                                                      |                                                 |                                      |
| Basic calcium petroleum sulfonate (180% excess base)                | 1.2                                             | 2                                    |
| Basic calcium C <sub>18-22</sub> alkyl salicylate (50% excess base) | 1.2                                             | 2                                    |
| "Santopoid S" (chloronaphtha methyl xanthate)                       | 3.0                                             | 5                                    |
| 2,6-ditertiarybutyl-4-methylphenol                                  | 0.3                                             | 0.5                                  |
| Phenyl-alpha-naphthylamine                                          | 0.06                                            | 0.1                                  |
| Yellow Dye (Sandoz Chem. Co.)                                       | 0.018                                           | 0.03                                 |
| Mineral Oil (100 SUS at 100° F.)                                    | 54.0                                            | 90.37                                |
| Water                                                               | Balance                                         | -----                                |
| Composition C:                                                      |                                                 |                                      |
| Basic barium petroleum sulfonate (50% excess base)                  | 1.2                                             | 2                                    |
| Basic barium C <sub>18-22</sub> alkyl salicylate (50% excess base)  | 1.2                                             | 2                                    |
| "Santopoid S" (chloronaphtha methyl xanthate)                       | 3.0                                             | 5                                    |
| 2,6-ditertiarybutyl-4-methylphenol                                  | 0.3                                             | 0.5                                  |
| Phenyl-alpha-naphthylamine                                          | 0.06                                            | 0.1                                  |
| Yellow Dye (Sandoz Chem. Co.)                                       | 0.018                                           | 0.03                                 |
| Mineral Oil (100 SUS at 100° F.)                                    | 54.0                                            | 90.37                                |
| Water                                                               | Balance                                         | -----                                |
| Composition D:                                                      |                                                 |                                      |
| Basic calcium dinonyl naphthalene sulfonate (50% excess base)       | 2                                               | 3.3                                  |
| Basic calcium cetyl salicylate (25% excess base)                    | 2                                               | 3.3                                  |
| Chloronaphthaamylxanthate                                           | 2                                               | 3.3                                  |
| Mineral Oil                                                         | 54                                              | 90.1                                 |
| Water                                                               | 40                                              | -----                                |
| Composition E:                                                      |                                                 |                                      |
| Basic calcium dinonyl naphthalene sulfonate (50% excess base)       | 2                                               | 3.3                                  |
| Basic calcium diwaxbenzoate (25% excess base)                       | 2                                               | 3.3                                  |
| Chloronaphthabutylxanthate                                          | 2                                               | 3.3                                  |
| Mineral Oil                                                         | 54                                              | 90.1                                 |
| Water                                                               | 40                                              | -----                                |

The outstanding properties which compositions of this invention possess are shown in Table I. The stability was determined by measuring the amount of water and oil separation at 140° F. from a 100 ml. test sample. The load carrying properties were determined on the Timken machine while the wear resistant properties of the emulsions were determined by measuring the amount of wear in a Vickers vane pump (Model V-104-A) while circulating the test fluid under conditions indicated in Table I. The fire-resistance was determined by the pipe cleaner test described in "Lubrication Engineering," March-April 1955, pages 86-87.

Table I

| Composition                                                                                                 | B   |        | X <sup>1</sup> |        | Y <sup>2</sup>              |       |
|-------------------------------------------------------------------------------------------------------------|-----|--------|----------------|--------|-----------------------------|-------|
|                                                                                                             | Oil | Water  | Oil            | Water  | Oil                         | Water |
| Emulsion Stability at 140° F.: Separation, Percent Vol.—                                                    |     |        |                |        |                             |       |
| 4 days                                                                                                      | 1   | trace  | 1              | trace  | 4                           | Trace |
| 13 days                                                                                                     | 3   | slight | 3              | slight | 25                          | 3     |
| 18 days                                                                                                     | 6   | slight | 6              | slight | complete separation         |       |
| Timken Test at 150° F./10 mm.: Failure Load, lb.                                                            |     | 20     |                | 5      |                             |       |
| Pump Wear Test: Total wear of Vanes and Ring Combined (300 hr. at 1,000 p.s.i. fluid temp. 150° F.), grams. |     | 0.165  |                | 0.200  | failed. 0.300 (at 100 hr.). |       |
| Equilibrium Wear Rate of Vanes and Ring Combined, grams/1,000 hr.:                                          |     |        |                |        |                             |       |
| 1,000 p.s.i.                                                                                                |     | 0.49   |                | 0.38   | failed.                     |       |
| 1,200 p.s.i.                                                                                                |     | 0.66   |                | 0.27   |                             |       |
| 1,500 p.s.i.                                                                                                |     | 0.75   |                | 8.4    |                             |       |
| 1,800 p.s.i.                                                                                                |     | 0.75   |                | failed |                             |       |

<sup>1</sup> Composition X [57% mineral oil (100 SUS at 100° F.)+1.2% basic calcium petroleum sulfonate+1.2% basic calcium C<sub>18-22</sub> alkyl salicylate+0.3% 2,6-ditertiarybutyl-4-methyl phenol+0.06% phenyl-alpha-naphthylamine+0.018% Yellow Dye+40% water].

<sup>2</sup> Composition Y [54% mineral oil+1.2% basic calcium petroleum sulfonate+1.2% basic calcium C<sub>18-22</sub> alkyl salicylate+0.3% 2,6-ditertiarybutyl-4-methyl phenol+0.06% phenyl-alpha-naphthylamine+3% Zn alkyl dithiophosphate+0.018% Yellow Dye+40% water].

The substitution of other wear inhibitors for the chloroxanthate in composition B of this invention, such as chlorinated paraffin wax, zinc cyclohexyl dithiophosphate or the zinc and cadmium salts of diamyl dithiocarbamic

acid resulted in compositions having poor emulsion stability and viscosity.

In the pipe cleaner test, compositions A through D passed over 50 cycles while mineral oil or mineral oil containing 4% of Ca petroleum sulfonates and/or Ca C<sub>12-22</sub> alkyl salicylate ignited after about 5 cycles.

Compositions of this invention are particularly suitable for use in diesel engines, in die casting machines, in permanent mold machines in steel mill equipment such as coke pushers, pipe coupling tighteners, combustion control mechanisms, plastic molding presses and glass blowing machines and the like.

We claim as our invention:

1. A water-in-oil emulsion lubricant and hydraulic fluid which is from about 20% to about 45% water phase and from about 55% to about 80% oil phase, the oil phase being essentially a mineral oil containing from about 0.5% to about 12% each, based on the oil, of an oil-soluble basic alkaline earth metal organic sulfonate and an oil-soluble basic alkaline earth metal alkyl salicylate from about 3% to about 10% of an oil-soluble chlorine-containing naphtha xanthate.

2. A water-in-oil emulsion lubricant and hydraulic fluid which is from about 20% to about 45% water phase and from about 55% to about 80% oil phase, the oil phase being essentially a mineral oil containing from about 2% to about 4% each, based on the oil, of an oil-soluble basic alkaline earth metal organic sulfonate and an oil-soluble basic alkaline earth metal alkyl salicylate and from about 3% to about 10% of an oil-soluble chlorine-containing naphtha xanthate.

3. The composition of claim 2 containing in the emulsion from 0.01% to 2% of an oil-soluble anti-oxidant selected from the group consisting of phenolic and aryl amine compounds.

4. A water-in-oil emulsion lubricant and hydraulic fluid which is from about 30% to about 40% water phase and from about 70% to about 60% oil phase, the oil phase being essentially a mineral oil containing from about 2% to about 4% each, based on the oil, of oil-soluble basic calcium petroleum sulfonate, and oil-soluble basic calcium C<sub>18-22</sub> alkyl salicylate and from about 3% to about 10% of oil-soluble polychloronaphtha xanthate.

5. The composition of claim 4 containing in the emulsion from about 0.01% to about 1% each of an oil-soluble alkylphenol and an oil-soluble arylamine.

6. A water-in-oil emulsion lubricant and hydraulic fluid

which is from about 40% water phase and about 60% oil phase, the oil-phase being essentially a mineral oil containing from about 1% to about 2% each of oil-soluble basic calcium petroleum sulfonate and oil-soluble

basic calcium  $C_{18-22}$  alkyl salicylate and from about 3% to about 10% of polychloronaphtha xanthate.

7. The composition of claim 6 containing in the emulsion from about 0.01% to about 1% each of 2,6-di-tert-butyl-4-methyl phenol and phenyl-alpha-naphthylamine.

8. A mineral oil concentrate composition adapted for making stable water-in-oil emulsion lubricant and hydraulic fluid consisting essentially of a mineral oil containing from about 0.5% to about 12% each of an oil-soluble basic alkaline earth metal petroleum sulfonate, oil-soluble basic alkaline earth metal  $C_{18-22}$  alkyl salicylate and oil-soluble polychloronaphtha xanthate.

9. A mineral oil concentrate composition adapted for making stable water-in-oil emulsion lubricant and hy-

draulic fluid consisting essentially of a mineral oil containing from about 0.5% to about 12% each of an oil-soluble basic calcium petroleum sulfonate, oil-soluble basic calcium  $C_{18-22}$  alkyl salicylate and oil-soluble polychloronaphtha xanthate.

References Cited in the file of this patent

UNITED STATES PATENTS

|    |           |                            |               |
|----|-----------|----------------------------|---------------|
| 10 | 2,153,495 | Berger et al. _____        | Apr. 4, 1939  |
|    | 2,153,496 | Berger et al. _____        | Apr. 4, 1939  |
|    | 2,466,647 | Stern _____                | Apr. 5, 1949  |
|    | 2,744,870 | Stillebroer _____          | May 8, 1956   |
|    | 2,820,007 | Van Der Minne et al. _____ | Jan. 14, 1958 |